

## UNITED STATES PATENT OFFICE

2,501,337

## TREATMENT OF CELLULOSIC FIBROUS MATERIALS

Hendrik Christiaan Jansen, Upton Park, Chester, and Newton Wood Barritt, Ince, near Chester, England, assignors to Shell Development Company, San Francisco, Calif., a corporation of Delaware

No Drawing. Application December 19, 1945, Serial No. 636,066. In Great Britain December 15, 1944

7 Claims. (Cl. 117—56)

1

This invention relates to a process for the treatment of fibrous materials.

It is an object of the present invention to provide an improved process for the wetting of fibrous materials, particularly those of a cellulosic nature such as cotton fibrous material, rayon, sisal and manila hemp.

According to the present invention, a process is provided for the wetting out of fibrous materials, particularly cellulosic material such as cotton fibrous material, wherein the material is first treated with a mono-oxy compound having the oxygen atom directly linked to a single carbon atom of a hydrocarbon radical of eight to eleven carbon atoms followed by a treatment with an aqueous solution of an anion active detergent or wetting agent such as a water-soluble salt of an organic compound in which a hydrocarbon radical is linked with a carboxylated, sulfonated or sulfated solubilizing group through an ester, amide or aryl linkage. Examples of such detergents which are commercially available are the salts of sulfonated or sulfated primary aliphatic alcohols (containing at least eight carbon atoms in the molecule) derived from fatty acid sources; the salts of sulfonated or sulfated secondary aliphatic alcohols (containing at least eight carbon atoms in the molecule) derived from synthetic sources such as petroleum; salts of isethionic acid or of taurine condensation products with fatty acids and salts of alkyl, aryl, aralkyl, alkaryl, or keryl sulfonates. The term "keryl," as used herein, refers to the radical of an aliphatic hydrocarbon obtainable from kerosene. Examples of the carboxylated type of detergent are: fatty acid, naphthenic or rosin acid soaps.

Preferably, the mono-oxy compound used in the first step of the process is an alcohol, most preferably a primary or secondary alcohol, or a mixture thereof having an average chain length of eight to eleven carbon atoms per molecule, and preferably the anion active compound used in the second step is a sulfated aliphatic alcohol detergent, most preferably a sodium salt of a sulfated aliphatic alcohol containing from eight to eighteen (and preferably sixteen to eighteen) carbon atoms in the molecule, or a mixture of such salts such as is obtained by the sulfation of a mixture of olefins containing from six to eighteen carbon atoms in the molecule. While the invention will

2

be particularly described with reference to the use in the first step of alcohols having an average chain length of eight to eleven, most preferably about nine, carbon atoms because of their outstanding superiority, it is also applicable to other mono-oxy compounds wherein the oxygen atom is linked to a single carbon atom of a hydrocarbon radical of eight to eleven carbon atoms, such as ketones and aldehydes.

10 It has already been proposed to improve the effective wetting power of alkyl sulfate salts by the use of higher aliphatic alcohols. Thus, U. S. Patents 2,166,314 and 2,166,315 show that such an improvement may be obtained by employing 15 an aqueous mixture of an alkyl sulfate salt and a higher alcohol, preferably an alcohol corresponding to the alkyl sulfate salt used. An important object of the present invention is to improve upon the prior methods of wetting out 20 fibrous material. More particularly, it is an object of the present invention to provide a more efficient and more economical method for carrying out such wetting operations. Another object is to materially reduce the wetting and treating 25 time of fibrous materials in kier boiling, dyeing and the like, and to improve the quality of the products of these operations, particularly with respect to uniformity. Still other objects and 30 advantages of the new process of the invention will be apparent from the following more detailed description thereof.

It has now been found that very greatly improved results may be obtained in wetting out 35 fibrous materials by pretreating the fibrous material with an alcohol, or other mono-oxy compound wherein the oxygen atom is directly linked to a single carbon atom of a hydrocarbon radical having an average length in the compound or mixture thereof used of eight to eleven carbon 40 atoms, before contacting the fibers with the aqueous wetting solution. Not only are the results markedly better than when the same oxy-compounds are used in conjunction with the aqueous wetting solution, but also they are greatly superior to those obtainable by pretreating the 45 fibrous material with other polar agents or even with other mono-oxy compounds of the same general character but having a different chain length.

While, as previously indicated, primary or sec-

secondary aliphatic alcohols having a straight hydrocarbon chain of eight to eleven carbon atoms, such as n-octyl alcohol, n-nonyl alcohol, n-decyl alcohol, n-undecyl alcohol, 2-octanol, 4-octanol, 3-nonenol, 2-decanol, 2-undecanol, etc., are the preferred pretreating agents, branched chain aliphatic alcohols, for example, 2-methyl-4-heptanol, 2,2,4-trimethyl-3-pentanol, 2,2,4-trimethyl-4-pentanol, 2,7-dimethyl-4-octanol, and the like, may also be used. Non-aliphatic alcohols can likewise be used as the pretreating agent in the process—3-phenyl propanol, p-ethyl benzyl alcohol, tertiary butyl cyclohexanol, terpineol, and the like being suitable, for example. Among the ketones which may be used are, for instance, methyl heptyl ketone, ethyl isoamyl ketone, isopropyl n-butyl ketone, diisobutyl ketone, isobutyl n-amyl ketone, isopropyl cyclohexanone, acetophenone, etc. Aldehydes such as octyl aldehyde, decyl aldehyde, etc., are also useful in the process. Unsaturated alcohols, ketones and aldehydes corresponding to the foregoing and like compounds may likewise be used. Examples of such compounds are: 2-octene-4-ol, 6-methyl-4-heptene-2-ol, 2,6-dimethyl-2-heptene-7-ol, 1-decene-4-ol, phorone, isophorone, cyclohexenylethanol, citronellol, and the like.

The mono-oxy compound may be used in pure or substantially pure form or as mixtures of one or more such individual compounds with or without other compounds which do not interfere with their desired action on the fibrous material being treated. Where mixtures of mono-oxy compounds of the indicated type are used, it is not essential that the individual components of the mixture used have hydrocarbon radicals of eight to eleven carbon atoms, provided the weighted average of such radicals falls in this range. In fact, an important feature of the invention is based upon the discovery that mixtures of a mono-oxy compound wherein the oxygen atom is attached to a single carbon atom of a hydrocarbon chain of less than eight carbon atoms with another mono-oxy compound having the oxygen atom attached to a single carbon atom of a hydrocarbon chain of more than eight carbon atoms, such that the average of the chain lengths is eight to eleven carbon atoms, show a synergistic effect in that better results may be obtained with the mixture than with either component alone. This is the case, for example, with a mixture of equal parts of secondary hexyl alcohol and secondary decyl alcohol. Other mixtures which may be similarly used are, for instance, n-amyl alcohol with secondary dodecyl or lauryl alcohol, mesityl oxide with lauryl alcohol or ethyl-octyl ketone, etc. However, it is desirable that all components of the treating mixture be substantially water-insoluble.

The chosen mono-oxy treating agent or mixture thereof may be applied to the fibrous material in various ways. For instance, the material may be exposed to vapors of the chosen alcohol, aldehyde and/or ketone until the surface of the fibers is uniformly covered with an adsorbed layer thereof. Alternatively, the treating agent may be applied as a spray or mist to the fibrous material. Immersion of the fibers in the liquid treating agent or in a suitable non-aqueous solution thereof, preferably in a volatile solvent, e. g. in an ethereal solution, may likewise be used to deposit the desired surface film of alcohol, aldehyde and/or ketone thereon. Where solvents are used in depositing the treating agent, they may advantageously be recovered for reuse be-

fore passing the pretreated fibrous material to the next step of the process, and in the interest of economy it is generally preferred to use liquid mono-oxy treating agents and to apply them directly to the fibers by diffusion or spreading, etc. without use of solvents.

The following tests show the advantages of the present invention.

#### EXAMPLE I

Eight hanks of cotton yarn were placed in a tin above filter papers on which 1 cc. of a higher secondary alcohol or ketone had been dropped. The tin was closed and allowed to stand for five hours at the temperature stated in the following table. The wetting power was measured by the Draves test (cf. American Dyestuff Reporter (1939), 28, 425).

For the test of the wetting power solutions containing between 0.02% and 0.15% of a mixture of sodium salts of secondary aliphatic sulfated alcohols containing from sixteen to eighteen carbon atoms in the molecule, hereinafter referred to as "ester salts" (obtained by sulfating a mixture of olefins containing from eight to eighteen carbon atoms in the molecule obtained by the cracking of paraffin wax), were used.

The wetting power is calculated in terms of the concentration of ester salt solution required to give a sinking time of 25 seconds, this concentration being expressed relative to that of a standard sample of ester salt solution and standard untreated cotton which gave a sinking time of 25 seconds at an ester salt concentration of 0.8 gm. per liter. Thus, if the treated hank required an ester salt solution of only 0.2 gm. per liter to give a sinking time of 25 seconds, the wetting power is said to be 400 relative to the standard sample which is assigned a wetting power of 100 by definition. The results are shown in Table I:

Table I

| Treating Agent                                      | Wetting Power    | Pretreatment Temperature, °C. |
|-----------------------------------------------------|------------------|-------------------------------|
| None                                                | <sup>1</sup> 100 | 23                            |
| Sec. Hexyl alcohol                                  | 109              | 23                            |
| Sec. Heptyl alcohol                                 | 320              | 23                            |
| Sec. Octyl alcohol                                  | 2,140            | 23                            |
| Sec. Nonyl alcohol                                  | 1,800            | 23                            |
| Sec. Decyl alcohol                                  | 1,120            | 23                            |
| Mixture of Sec. Undecyl and Dodecyl alcohols (1:1)  | 115              | 23                            |
| Mixture of Sec. Undecyl and Dodecyl alcohols (1:1)  | 800              | 40                            |
| Mixture of Sec. Hexyl and Sec. Decyl alcohols (1:1) | 1,900            | 23                            |
| Di-isobutyl ketone                                  | 880              | 20                            |
| Methyl-heptyl ketone                                | 1,200            | 20                            |

<sup>1</sup> By definition.

#### EXAMPLE II

The following results have been obtained with fatty acid soaps:

A domestic fatty acid soap no activating substance: Wetting power 55 at 40° C.

55 Same domestic fatty acid soap activation with mixed sec. octyl and nonyl alcohol: Wetting power 100 at 40° C.

At 25° C. the sinking time for an 0.05% solution of the same soap, improved from 720 seconds to 56 seconds, after pretreatment of the hanks with mixed secondary octyl and nonyl alcohol vapors.

Very much poorer results are obtained by mixing the secondary alcohol with the aforesaid

ester salts solutions as described in U. S. Patents 2,166,314 and 2,166,315. Table II shows the inefficiency of such a procedure as compared with the process described in the present application.

Table II

| Activating Substance                       | Percent by wt. added | Wetting Power |
|--------------------------------------------|----------------------|---------------|
| Nil                                        |                      | 100           |
| Sec. Hexyl alcohol                         | 4                    | 101           |
| Sec. Heptyl alcohol                        | 4                    | 115           |
| Sec. Octyl alcohol                         | 4                    | 218           |
| Mixture of Sec. Octyl and Nonyl alcohols   | 4                    | 253           |
| Mixture of Sec. Decyl and Dodecyl alcohols | 4                    | 213           |

<sup>1</sup> By definition.

The superiority of the process of the invention over even pretreatment with other polar compounds is shown by the following results obtained by following the same procedure as in Example I, using a treating temperature of about 23° C.:

Table III

| Pretreating Agent     | Wetting Power of Ester Salt Solution by Draves Test |
|-----------------------|-----------------------------------------------------|
| Glycerol              | 90                                                  |
| Ethyleneglycol        | 100                                                 |
| Di-acetone alcohol    | 100                                                 |
| Cyclohexanol          | 90                                                  |
| Di-methylphthalate    | 120                                                 |
| Di-butylphthalate     | 110                                                 |
| Methylisobutyl ketone | 140                                                 |
| Nitrobenzene          | 110                                                 |
| Aniline               | 140                                                 |
| Furfural              | 130                                                 |
| Pinetar               | 120                                                 |
| Di-isopropyl ether    | 130                                                 |

It will thus be seen that the invention offers many advantages over prior art methods of wetting out fibrous materials, particularly with respect to economy in the use of treating agents. The process is capable of wide variation not only with regard to the mono-oxy compounds having the oxygen atom attached to a single carbon atom of a hydrocarbon radical of eight to eleven carbon atoms which may be used, but also in relation to the method of applying the film of pretreating agent to the fibers in the pretreatment step of the invention. It will therefore be understood that the process is not limited to the materials or methods described by way of illustration of the principles involved, nor by any theory proposed in explanation of the improved results attained.

We claim as our invention:

1. In a process of treating cellulosic fibrous material wherein the fibers are wetted with an aqueous solution of an anion-active wetting agent, the improvement which comprises the step of preliminarily treating the fibers with a substantially water-insoluble mono-oxy substituted hydrocarbon treating agent containing only carbon, hydrogen and oxygen in the molecule, said agent selected from the group consisting of the aliphatic alcohols, aliphatic ketones and aliphatic aldehydes having 8 to 11 carbon atoms per molecule and mixtures of at least two members of the group consisting of aliphatic alcohols, aliphatic ketones and aliphatic aldehydes having an average of 8 to 11 carbon atoms per molecule in the mixture to deposit on said fibers a surface film of said treating agent before carrying out said wetting of the fibrous material.

2. In a process of treating cellulosic fibrous material wherein the fibers are wetted with an aqueous solution of an anion-active wetting agent, the improvement which comprises the step of preliminarily treating the fibers with at least one aliphatic secondary mono-hydroxy alcohol having a hydrocarbon radical of 8 to 11 carbon atoms per molecule and containing only carbon and hydrogen atoms and one oxygen atom in the molecule to deposit on the fibers a surface film of said alcohol before carrying out said wetting of the fibrous material.
3. In a process of treating cellulosic fibrous material wherein the fibers are wetted with an aqueous solution of an anion-active wetting agent, the improvement which comprises the step of preliminarily treating the fibers with at least one aliphatic mono-ketone having the keto-oxygen atom directly attached to a hydrocarbon radical of 8 to 11 carbon atoms, said ketone containing only carbon and hydrogen atoms and one oxygen atom in the molecule to deposit on the fibers a surface film of said ketone before carrying out said wetting of the fibrous material.
4. In a process of treating cellulosic fibrous material wherein the fibers are wetted with an aqueous solution of an anion-active wetting agent, the improvement which comprises the step of preliminarily treating the fibers with a mixture of substantially water insoluble aliphatic monohydroxy alcohols containing only carbon and hydrogen atoms and one oxygen atom in the molecule, one of which alcohols contains less than 8 carbon atoms and another of which alcohols is of higher molecular weight such that the average number of carbon atoms per molecule of the mixture is 8 to 11 to deposit on the fibers a surface film of said alcohol mixture before carrying out said wetting of the fibrous material.
5. In a process of treating cotton fibers wherein the fibers are wetted with an aqueous solution of a sodium alkyl sulfate of 8 to 18 carbon atoms per molecule, the improvement which comprises the step of exposing the fibers to the vapors of a mixture of at least one substantially water insoluble aliphatic secondary mono-hydroxy alcohol having less than 8 carbon atoms per molecule together with at least one aliphatic secondary mono-hydroxy alcohol having more than 8 carbon atoms per molecule in proportions such that the average number of carbon atoms per molecule in the mixture is 8 to 11, said alcohols containing only carbon and hydrogen atoms and one oxygen atom in the molecule, whereby a film of said alcohols is deposited on the fibers before said wetting of the fibers is carried out.
6. In a process of treating cotton fibers wherein the fibers are wetted with an aqueous solution of a sodium alkyl sulfate of 8 to 18 carbon atoms per molecule, the improvement which comprises the step of exposing the fibers to the vapors of a mixture of at least one substantially water insoluble dialkyl ketone having less than 8 carbon atoms per molecule together with at least one dialkyl ketone having more than 8 carbon atoms per molecule in proportions such that the average number of carbon atoms per molecule in the mixture is 8 to 11, said ketones containing only carbon and hydrogen atoms and one oxygen atom in the molecule, whereby a film of said ketones is deposited on the fibers before said wetting of the fibers is carried out.
7. A process of treating cellulosic fibrous material which comprises exposing said fibers to the

vapors of a substantially water-insoluble mono-oxy substituted hydrocarbon treating agent containing only carbon, hydrogen and oxygen in the molecule, said agent selected from the group consisting of the aliphatic alcohols, aliphatic ketones and aliphatic aldehydes having 8 to 11 carbon atoms per molecule and mixtures of at least two members of the group consisting of aliphatic alcohols, aliphatic ketones and aliphatic aldehydes having an average of 8 to 11 carbon atoms per molecule in the mixture until a film of said agent is deposited on the fibers and subsequently contacting the thus treated fibers with an aqueous solution of an anion-active wetting agent.

15

HENDRIK CHRISTIAAN JANSEN.  
NEWTON WOOD BARRITT.

## REFERENCES CITED

The following references are of record in the file of this patent:

## UNITED STATES PATENTS

|    | Number    | Name          | Date          |
|----|-----------|---------------|---------------|
| 5  | 2,062,504 | Chapman       | Dec. 1, 1936  |
|    | 2,166,314 | Martin        | July 18, 1939 |
|    | 2,166,315 | Martin        | July 18, 1939 |
| 10 | 2,168,286 | Eustis et al. | Aug. 1, 1939  |
|    | 2,344,671 | Bertsch       | Mar. 21, 1944 |